

## UNITED STATES PATENT OFFICE

2,285,430

## LITHOGRAPHIC INK

Albert E. Gessler, New York, N. Y., Everett F. Carman, Dumont, N. J., and Louis F. Engelhart, Rockville Centre, N. Y., assignors to Interchemical Corporation, New York, N. Y., a corporation of Ohio

No Drawing. Application June 30, 1937,  
Serial No. 151,174

4 Claims. (Cl. 106—32)

This invention relates to lithographic inks and provides a new ink for lithographic printing which permits the speeding up of lithographic printing processes and makes possible for the first time lithographic web printing on non-absorbent material. Our new invention is especially valuable for lithographic printing on metal.

Lithographic offset printing is now generally used for printing on sheet metal to be used for making tin cans and other containers. The drying oil inks used in the process are set by oxidation and polymerization. It is customary to accelerate the setting by heating from 200—300° F., but, even under these circumstances, a period of from 20 to 30 minutes is required to set the ink. This requires bulky furnaces and mechanism for stacking the printed metal sheets in the furnaces and precludes the possibility of web printing.

While there has long been a demand for a quick-drying lithographic ink which would do away with the delay and inconveniences of the present method, it has heretofore proved impossible to provide an ink of reasonable cost which would meet the numerous physical requirements for an ink satisfactory for lithographic offset printing without introducing substantial quantities of drying oils which cannot be set rapidly. By our invention, we have, we believe for the first time, produced an ink which meets all the requirements of lithographic printing and which also has the ability to stand very high temperatures without injury and to set almost instantaneously at such temperatures. The use of this ink entirely does away with the necessity of the cumbersome furnaces now used in connection with lithographic printing on metal, and makes it possible to substitute a furnace of small dimensions heated to a high temperature through which the sheets may be passed horizontally, for the time of heating required is reduced from a period of 20 to 30 minutes to a matter of 2 or 3 seconds. Furthermore, the use of our ink permits passing the sheet metal through the press and also through the furnace in web form, thus facilitating the handling of the metal in speeding up the process.

A lithographic ink embodying our invention has a vehicle consisting of a water-repellant natural or synthetic resin dissolved in a volatilizable solvent consisting of paraffin hydrocarbons substantially free from unsaturated and aromatic constituents. The vapor pressure of the solvent is such that it is substantially non-volatile at room temperatures, while it evaporates

with great rapidity when exposed to high temperatures such as 1000—2000° F.

A further feature of the invention, which is particularly important in metal printing, consists in plasticizing the resin of such an ink by a plasticizer which is substantially non-volatile when exposed to high temperatures, such as 1000—2000° F., so that, after the ink has been exposed to such temperatures to evaporate the solvent, the plasticized resin remains uninjured and gives the ink film sufficient plasticity to avoid cracking when the printed metal is made up into containers.

An ink embodying our invention has all the physical and chemical properties necessary for good offset lithographic printing.

In the first place, it has no tendency to emulsify with the water or usual fountain liquids used on lithographic presses. The resin used as a binder is a water-repellant substance such as a rosin ester, a polymerized hydrocarbon, a modified alkyd resin, a phenolic resin, a damar resin, or the like. The plasticizer used with the resin is also water-repellant. It may be a vegetable or animal oil, such as peanut, soya, linseed, corn and fish oil, or an ester, such as methyl abietate, tricresyl phosphate; or plastic synthetic resins, such as oil-modified alkyds, may be used. The solvent, consisting of paraffin hydrocarbons, is also water-resistant. The result of this selection of the binder and solvent is that the solution forming the vehicle of the ink is highly water-repellant and shows no tendency to emulsify either with water alone or with the various conventional fountain liquids which include various dilute solutions of water-soluble substances.

In the next place, the ink is stable on the press and maintains the proper consistency for good offset lithographic printing. By proper portioning of the resin to the solvent, the desired stiff consistency of the present linseed oil lithographic inks can easily be obtained. The maintaining of this consistency on the press over long periods is the result of several factors. One is the high boiling point of the solvent which renders it substantially non-volatile at ordinary room temperatures (60—90° F.). This result is attained by using a hydrocarbon mixture not more volatile than is indicated by a 5% distillation at 200° C. and a 95% distillation at 220° C.

This factor alone, however, is not sufficient to secure the required stability of consistency. The chemical composition of the vehicle is also of great importance, for the ink must be spread out on inking rollers on the press and then offset

from the printing member to a blanket. In the past, rollers and blankets were made almost entirely of rubber; but the oils in ordinary lithographic inks have an appreciable swelling action on rubber, so that rubber rollers and blankets have a rather short life. Rubber rollers have been almost entirely replaced by composition rollers, made of polymerized oils, which are much more resistant to oil swelling; while compositions have been introduced for the blankets (such as compositions made with Thiokol, a plastic made by treatment of halogenated olefines with polysulfides) which are much more enduring than rubber blankets. We have found that if the ink has any tendency to react with, absorb, or to be absorbed by, these materials used in the usual rollers and blankets of a lithographic press, it will fail to give proper printing over long periods and be of no practical value. These difficulties are avoided in our ink by the use of paraffin hydrocarbons substantially free from any unsaturated or aromatic hydrocarbons. The solvent used in our ink is a petroleum distillate or chemical cut which has been treated to remove unsaturated and aromatic constituents. Our solvent most desirably is so free from such constituents that it has a dimethyl sulphate value of 1.0 or less (the dimethyl sulphate value is obtained by mixing 100 cc. of the solvent with 100 cc. of dimethyl sulphate, the percentage of the solvent soluble in the dimethyl sulphate being the dimethyl sulphate value). A dimethyl sulphate value exceeding 4.0 or 5.0 indicates that a hydrocarbon mixture is unsuitable for use in our ink. Small amounts of certain additions may be included in such solvents, provided they do not substantially increase the swelling action of the mixture on the rollers; thus, we have found that certain higher alcohols, e. g. lauryl alcohol, can be used in amounts up to a very few percent, without increasing the solvent action of the hydrocarbons.

In addition to meeting the requirements for offset lithographic printing, our ink has the ability to stand very high temperatures without injury and to set substantially instantaneously at such temperatures. To insure instantaneous setting, we use a hydrocarbon mixture which is completely volatilized at a temperature not exceeding 400° C. Substantially instantaneous volatilization of such solvents may be obtained by exposing the prints to temperatures of the order of 1000-2000° F. for a period of a few seconds. In such treatment, the prints do not reach the temperatures of the oven; the print temperatures probably never go above 300° C. The non-volatility of the plasticizer at these temperatures prevents the intense heat from injuring the ink and leaves the resin adequately plasticized after such temperatures have been used to evaporate the solvent.

In its preferred form, our ink is capable, after setting, of adhering to metal sheets without cracking when these sheets are bent to form them into containers. This result is obtained by use with the resin of a water-resistant, non-volatile plasticizer in a quantity sufficient to give the plasticized resin a plasticity of at least .026 centimeters, using a standard A. S. T. M. penetrometer with a standard needle and a 200 gram weight acting on the needle for 60 seconds at 25° C.

The following are typical examples of inks made in accordance with our invention:

**EXAMPLE 1.—Clear lithographic varnish**

|                                                                                                   |      |
|---------------------------------------------------------------------------------------------------|------|
| Ester gum (rosin, substantially completely esterified with glycerol)                              | 50.4 |
| 5 Oil modified alkyd resin (Duraplex C 45                                                         |      |
| L. V.—Resinous Products Co.)                                                                      | 11.4 |
| Paraffin hydrocarbons (272-311° C.)                                                               | 38.2 |
| (The boiling range of all of our hydrocarbons is shown from 5% distillation to 95% distillation.) |      |

This clear varnish is intended for use in overprinting an ink lithographically, to protect the print and increase the gloss. The formula is especially intended for tin printing, as sufficient alkyd resin plasticizer is present to permit of forming after drying.

**EXAMPLE 2.—Red ink**

|                                                     |      |
|-----------------------------------------------------|------|
| Lithol red                                          | 35   |
| Ester gum                                           | 34.3 |
| 20 Oil modified alkyd (Rezyl 869—American Cyanamid) | 7.8  |
| Paraffin hydrocarbons (272-311° C.)                 | 22.3 |
| Similar to above, for tin decorating.               |      |

**EXAMPLE 3.—Red ink**

|                                           |      |
|-------------------------------------------|------|
| 25 Barium lithol toner                    | 35.0 |
| Ester gum                                 | 39.0 |
| Peanut oil (plasticizer for tin forming)  | 7.8  |
| Paraffin hydrocarbons (B. P. 263-297° C.) | 18.2 |

**EXAMPLE 4.—Yellow ink**

|                                                         |      |
|---------------------------------------------------------|------|
| Chrome yellow                                           | 55.1 |
| Hansa yellow                                            | 3.6  |
| Aluminum hydrate                                        | 7.4  |
| Varnish                                                 | 33.9 |
| 35 Phenolic resin (Amberol ST137 Resinous Products Co.) | 53.0 |
| Oil modified alkyd resin (Glyptal 2464—G. E.)           | 12.0 |
| Paraffin hydrocarbon (283-326 C.)                       | 35.0 |

**EXAMPLE 5.—Blue ink**

|                                                                      |      |
|----------------------------------------------------------------------|------|
| Iron blue                                                            | 40   |
| Varnish                                                              | 60   |
| Modified maleic anhydride resin (Paranol 45 89—Paramet Chemical Co.) | 57.0 |
| Peanut oil                                                           | 12.0 |
| Paraffin hydrocarbon (B. P. 272-311° C.)                             | 31.0 |

**EXAMPLE 6.—White ink**

|                                                     |    |
|-----------------------------------------------------|----|
| 50 Titanium dioxide                                 | 55 |
| Zinc oxide                                          | 5  |
| Modified maleic anhydride resin (Paranol 89)        | 26 |
| Peanut oil                                          | 5  |
| 55 Paraffin hydrocarbon mixture (B. P. 300-360° C.) | 19 |

**EXAMPLE 7.—Black ink**

|                                              |    |
|----------------------------------------------|----|
| Carbon black                                 | 20 |
| 60 Iron blue                                 | 5  |
| Alkali blue                                  | 5  |
| Varnish                                      | 70 |
| Ester gum                                    | 59 |
| Oil modified alkyd                           | 13 |
| 65 Paraffin hydrocarbons (B. P. 272-311° C.) | 28 |

The method of application of these inks is substantially similar to the method of applying the old type lithographic inks; and they may be dried by the old methods. When run through a regular tin-lithographing set-up, our inks will dry in from 3 to 5 minutes, as compared to a 20 to 30 minute drying schedule for the old type inks.

75 With prints of our inks, almost instantaneous

drying may be obtained by evaporating the solvent, by exposing the printed surfaces to extremely high temperatures, of the order of 1000-2000° F., it being possible under such conditions to obtain complete drying in a time as short as from one to two seconds, as compared with a minimum of 20 minutes for the ordinary type of lithographic ink. It is possible to obtain complete drying in a continuous oven only 6 feet long, as compared with an 80 foot oven required for old style drying, even when accompanied by racking of the sheets. Thus it is possible to save both space and the labor required for racking and unracking.

Web printing of lithographic inks has been heretofore attempted on absorbent paper stock; even with absorbent paper, smudging and set-off occur because the ink is only partly absorbed and not really dry on the sheet. It has been impossible to print webs of fully sized paper, metal or non-absorbent stock from lithographic plates with inks heretofore available. Still another advantage of our inks is the fact that they can be dried sufficiently rapidly to permit of such web printing, either on paper or metal, without smudging or set-off.

Where a combustible material is printed with our inks, the heat necessary for drying should preferably be supplied to the paper by burners situated above the printed side of the paper. Direct flame ribbon burners or radiant heat burners may be employed. In this case, the paper itself will not attain a temperature sufficient to cause scorching, if proper precautions are taken as to web speed. With non-combustible materials, the heat may be applied in any convenient manner. The solvent may be merely evaporated, or it may be burned during the evaporation to insure a more complete removal of solvent.

The term "lithography", as used throughout the specification and claims, is the term as commonly used in the printing trade; it includes any

offset printing from planographic plates, whether stone or metal, flat or curved.

We claim:

1. A lithographic printing ink comprising pigment dispersed in a vehicle comprising a solvent consisting essentially of a petroleum fraction with a dimethyl sulfate value less than 4.0, which fraction is substantially non-volatile at about 90° F., but evaporates rapidly when exposed to a temperature of 1000°-2000° F. for a few seconds, and sufficient resin in said solvent to give the consistency of ordinary lithographic printing inks.
2. A lithographic printing ink comprising pigment dispersed in a vehicle comprising a solvent consisting essentially of a petroleum fraction with a dimethyl sulfate value less than 1.0, which fraction is substantially non-volatile at about 90° F., but evaporates rapidly when exposed to a temperature of 1000°-2000° F. for a few seconds, and sufficient resin in said solvent to give the consistency of ordinary lithographic printing inks.
3. A lithographic printing ink vehicle comprising a solvent consisting essentially of a petroleum fraction with a dimethyl sulfate value less than 4.0, which fraction is substantially non-volatile at 90° F., but evaporates rapidly when exposed to a temperature of 1000°-2000° F. for a few seconds, and sufficient resin in said solvent to give the consistency of ordinary lithographic printing ink vehicles.
4. The composition of claim 1 with the addition of a plasticizer which does not evaporate when exposed to a temperature of 1000°-2000° F. for a few seconds and which gives the resin a plasticity of at least .026 centimeters as measured on a standard A. S. T. M. penetrometer at 25° C., using a standard needle, a 200 gram weight and 60 seconds' time.

ALBERT E. GESSLER.  
LOUIS F. ENGELHART.  
EVERETT F. CARMAN.